

Jan. 25, 1927.

1,615,423

H. G. WALKER

METHOD AND APPARATUS FOR COATING CORES

Filed Feb. 26, 1923

2 Sheets-Sheet 1



Fig. 1.



Fig. 2.

Inventor  
Howard G. Walker  
by H. G. Patterson  
Atty.

Jan. 25, 1927.

1,615,423

H. G. WALKER

METHOD AND APPARATUS FOR COATING CORES

Filed Feb. 26, 1923

2 Sheets-Sheet 2

Fig. 3.



Fig. 4.



Fig. 5.



Fig. 6.



Fig. 7.



Fig. 8.



Inventor  
Howard G. Walker

by *Al Patterson*  
Atty.

## UNITED STATES PATENT OFFICE.

HOWARD GEORGE WALKER, OF BERRWYN, ILLINOIS, ASSIGNOR TO WESTERN ELECTRIC COMPANY, INCORPORATED, OF NEW YORK, N. Y., A CORPORATION OF NEW YORK.

## METHOD AND APPARATUS FOR COATING CORES.

Application filed February 26, 1923. Serial No. 621,242.

This invention relates to a method and apparatus for coating cores.

The object of the invention is to produce a core having a coating of pulp thereon which is attached to the core solely by the intermingling of the fibers thereof and without the use of any adhesive substance.

Briefly, the method consists in depositing pulposous material upon a foraminous member, bringing the core to be coated into contact with the deposited pulp on the foraminous member, depositing an additional amount of pulp on the core and on the foraminous member, bringing the core and pulp on the foraminous member into contact with a carrier, preferably a felt, transferring the pulp and core from the foraminous member to the carrier, removing the pulp and core from the carrier, and forming the pulp around the core so as to constitute a homogeneous coating therefor.

The present method may be employed to advantage for insulating electrical conductors, but it is to be understood that it is not limited to this purpose but only in so far as is defined by the appended claims. Where the method is used for insulating electrical conductors manila, wood, rag, cotton, esparto, jute, hemp, and asbestos pulps may be employed as the coating material, but other materials than those specified may be used without departing from the spirit and scope of the present invention, which contemplates in its broadest aspect the coating of any core with any pulp.

The drawings illustrate an apparatus by which the method may be practiced, the apparatus being especially designed for coating a core in strand form, but it is to be understood that other apparatus may be devised for coating cores in other forms without departing from the spirit and scope of the invention.

The word "pulp" as used in the specification and claims is to be understood as defining and including any cohering, fibrous mass whether suspended in a liquid, moist, or substantially dry.

In the accompanying drawings:

Fig. 1 is a side elevation of a preferred apparatus for performing the process;

Fig. 2 is an enlarged top plan view of the apparatus shown in Fig. 1, parts being omitted for the sake of clearness;

Fig. 3 is an enlarged fragmentary top

plan view showing the felt carrier for receiving the pulposous material from the foraminous member;

Fig. 4 is an enlarged fragmentary perspective view showing the manner in which the pulposous material is deposited on the foraminous member and on the core;

Figs. 5 and 6 are enlarged views showing the form of the pulp coating on the core as it is delivered from the carrier and the squeezing rolls respectively;

Figs. 7 and 8 are enlarged views showing the form of the pulp coating on the core during the forming operation and after the forming operation is completed respectively.

The steps of the method will be readily understood from a detailed description of the apparatus by which the method may be practiced.

Referring to the drawings in detail in which like reference numerals designate similar parts throughout the several views, a core to be coated is fed from a supply roll 10 over an idler roll 11 and thence around a drum 12 which is partly submerged in a liquid containing pulp within a semi-spherical trough 13.

The drum 12 may be of any suitable type, preferably comprising a pair of sheet metal sides 14 (Fig. 4) and a peripheral portion 15 secured thereto. The portion 15 is provided with a plurality of relatively large perforations 16 which are covered with a strip of fine wire mesh 17. The drum has a central tubular axle 18 which is rotatably mounted in suitable bearings 19 carried by the framework 20 which supports all of the elements of the apparatus. The level of the pulp mixture within the drum 12 is maintained at a lower level than that of the pulp in the tank 13, as indicated by dotted lines A and B respectively. This difference in levels is maintained by a siphon pipe 21 which has its inlet submerged in the drum 12 and its discharge through the tubular axle. A continuous circulation of the pulp mixture is maintained within the tank by feeding the pulp mixture from a supply pipe 22 which may be connected to a supply tank (not shown) into the tank 13, out of the said tank by a pipe 23 into a receiving tank (not shown) from which it is pumped back into the supply tank in any suitable manner. As the drum 12 revolves in the tank, due to the difference in levels

100  
105  
110

of the liquids in the drum and tank, the liquid will pass through the fine wire mesh, straining pulp onto the surface of the wire mesh.

5 Attention is called to the fact that the idler roll 11 is so spaced from the periphery of the drum 12 that the core is held out of contact with that section of the foraminous portion which is near the surface of the liquid in the tank, whereby pulp is strained onto said section of the foraminous portion before the strand is brought into contact therewith. The first deposit of pulp on the foraminous portion is indicated by 10 the letter C (Fig. 4). As the drum revolves in the tank, an additional amount of pulpy material will be deposited on top of the core and also upon the foraminous portion of the drum, forming a thicker coating indicated 15 by the letter D in Fig. 4. The drum 12 is rotated in the direction indicated by the arrow and the pulp on the foraminous portion 17 thereof together with the core are brought into contact with a felt covered roll 20 20. The periphery of the roll 24 has a foraminous portion formed of fine wire mesh 25 covered by felt 26, as shown in detail in Fig. 3, and as the pulp on the foraminous portion of the drum is brought into contact therewith, the "free liquid" so to speak, in 25 the pulp mixture will be squeezed out partially through the foraminous portion of the drum and partially through the felt and foraminous portion of the roll 24. The partially dried pulp adheres to the felt in the form of a ribbon with the core substantially centrally located therein as shown in Fig. 5, and the core with the pulp ribbon attached 30 passes around the roll 24 and between it and a second felt covered roll 27.

The rolls 24 and 27 are carried by a suitable bracket 28 supported by the framework 20, the roll 24 being positioned to engage the foraminous portion of the drum 12 with a 45 slight pressure. The rolls 24 and 27 are forced together by any suitable tension means which is adjustable to exert the proper pressure between the core and pulp ribbons as they pass between the rolls, this pressure serving to mat the pulpy material and secure it to the core to such an extent that as the core leaves the rolls it will carry the 50 pulp ribbon with it.

From the rolls 24 and 27 the core with its 55 pulp ribbon attached is passed between a pair of squeezing rolls 29 and 30, which are also forced together by any suitable means which is adjustable to present the proper pressure on the core and pulp ribbons as they pass 60 between the rolls, these rolls serving to remove additional moisture from the pulp ribbon and to more firmly mat the fibers of the ribbon and attach it to the core. The construction of the pulp coating as it leaves the 65 squeezing rolls 29 and 30 is shown in Fig. 6.

From the squeezing rolls the core with its ribbon pulp coating is drawn through a former which wraps the projecting edges of the ribbon around the core and around each other, the appearance of the coating after 70 it is first acted on by the former and after the forming action is completed being shown clearly in Figs. 7 and 8 respectively. The former causes a thorough intermingling of the pulp fibers and shapes the coating so that 75 it embraces the core and conforms to the shape thereof. This step of the process forms the coating into a mass so homogeneous that upon cutting the core and coating, the latter will not fray or ravel and will 80 not become easily detached from the core.

The former, indicated by the reference numeral 35, is illustrated as being of the same type as that fully shown and described in a co-pending application of Walker and 85 March, Serial No. 547,923, filed March 29, 1922. Reference is made to this application for a full disclosure thereof.

The former comprises essentially two plates 41 and 42 which wrap the projecting 90 edges of the pulp ribbon around each other and around the core in much the same manner as though the core and pulp ribbon were rolled on a table top with the palm of the 95 hand.

The core with its formed coating is drawn from the former and subjected to a mechanism for thoroughly drying out the coating. The means shown for performing this step in the process are a pair of wide hollow 100 drums 51 and 52 heated internally and having a plurality of grooves 53 formed thereon (Fig. 2), which receive the core, guides (not shown) being provided for directing the core over first one drum and then the other until 105 it has traversed all of the grooves on both drums, after which it is stored on a receiving drum 54. The drums 51 and 52 are revolvably mounted in suitable bearings carried by vertical standards supported by the 110 framework. The receiving drum 54 is also revolvably mounted in bearings carried by brackets 55 supported by the framework 20, and is driven by a motor 56 through suitable belting, the drums 51 and 52 being 115 driven from the drum 54 also through a suitable belting system.

Although it has been stated that the primary object of the invention is to apply a 120 coating of pulp to a core without the use of any adhesive substance, the process herein disclosed may be used with a pulp mixture containing a sizing substance, or the pulp may be deposited on a core which has been 125 previously treated with an adhesive agent, without departing from the spirit and scope of the present invention.

What is claimed is:

1. A method of coating a core in strand 130 form with pulp, which consists in collecting

pulpous material from liquid suspension, positioning the core adjacent said material, depositing additional pulpous material on the core, transferring the core and all of 5 said pulpous material to a carrier, removing said material from the carrier and then forming the material on the core to constitute a coating thereon.

2. A method of coating a core in strand 10 form with pulp, which consists in collecting wet, pulpous material from liquid suspension, placing the core adjacent said material, depositing additional wet, pulpous material on the core, transferring the core and 15 all of said pulpous material to a carrier and simultaneously removing some of the moisture from said material, removing said material from the carrier, forming the material on the core to constitute a coating thereon, 20 and then removing substantially all the moisture from said material.

3. A method of coating a core in strand form with pulp, which consists in forming a sheet of wet, pulpous material from liquid 25 suspension, positioning the core adjacent said sheet of material, depositing additional wet, pulpous material on the core, transferring the core and all of said pulpous material to a carrier and simultaneously 30 removing some of the moisture from said material, removing said material from the carrier, forming said material around the core to form a homogeneous coating therefor conforming with the shape of the core, 35 and then removing substantially all the moisture from said material.

4. A method of coating a core in strand form with pulp, which consists in collecting pulpous material from liquid suspension, 40 positioning the core adjacent said material, depositing additional pulpous material on said core, transferring the core and all of the pulpous material to a moving felt, removing said material from said felt and 45 then forming the material on the core to constitute a coating thereon.

5. A method of coating a core in strand form with pulp, consisting in forming a ribbon of pulpous material from liquid 50 suspension, placing the core adjacent said material, depositing additional pulpous material on the core and on said ribbon, transferring the core and said pulpous ribbon to a carrier, removing said material from the 55 carrier and then forming the material on the core to constitute a coating thereon.

6. A method of coating a core in strand form with pulp, consisting in depositing from a liquid suspension of pulp a ribbon 60 of wet pulpous material on a foraminous member, placing the core adjacent said deposited material, depositing additional wet pulpous material on the core and on said ribbon, transferring the core and said pulpous 65 ribbon from the foraminous member

to a carrier, removing said material from the carrier and then forming the material on the core to constitute a coating thereon.

7. A method of coating a core with pulp, 70 which consists in depositing from a liquid suspension of pulp a ribbon of wet pulpous material on a foraminous member, placing the core adjacent said pulpous material, depositing additional wet pulpous material on the core and on said ribbon, transferring 75 the core and said pulpous ribbon from the foraminous member to a carrier and simultaneously removing some of the moisture from said ribbon, and then removing said ribbon from the carrier and wrapping it 80 around the core to form a homogeneous coating therefor.

8. A method of coating a core with pulp, 85 which consists in depositing from a liquid suspension of pulp a ribbon of wet pulpous material on a foraminous member, placing the core adjacent said pulpous material, depositing additional wet pulpous material on the core and on said ribbon, transferring 90 the core and said pulpous ribbon from the foraminous member to a carrier and simultaneously removing some of the moisture from said ribbon, removing said ribbon from the carrier and wrapping it around 95 the core to form a homogeneous coating therefor, and then removing substantially all of the moisture from said coating.

9. A method of coating a core with pulp, 100 which consists in forming a ribbon of pulpous material from liquid suspension, placing the core adjacent said material, depositing additional pulpous material on the core and on the ribbon, transferring the core and said ribbon to a moving felt, and then removing said material from the felt.

10. A method of coating a core with pulp, 105 which consists in forming a ribbon of pulpous material from liquid suspension, placing the core adjacent said material, depositing additional pulpous material on the core and the ribbon, transferring the core and said ribbon to a moving felt, removing said material from the felt, and then wrapping said ribbon around said core to constitute a 110 homogeneous covering therefor.

11. A method of coating a core in strand form with pulp, which consists in forming a ribbon of wet pulpous material from liquid suspension, placing the core adjacent 115 said material, depositing additional wet pulpous material on the core and on said ribbon, transferring the core and said ribbon to a carrier, and simultaneously removing some of the moisture from said ribbon, removing an additional amount of moisture from said ribbon and then forming the material on the core to constitute a 120 coating thereon.

12. A method of coating a core with pulp, 125 which consists in forming a ribbon of wet

pulpous material from liquid suspension, placing the core adjacent said material, depositing additional wet pulpous material on the core and on said ribbon, transferring the core and said ribbon to a carrier, and simultaneously removing some of the moisture from said ribbon, removing an additional amount of moisture from said ribbon, and then wrapping said ribbon around the core to form a homogeneous coating therefor.

13. A method of coating a core with pulp, which consists in forming a ribbon of wet pulpous material from liquid suspension, placing the core adjacent said material, depositing additional wet pulpous material on the core and on said ribbon, transferring the core and said ribbon to a carrier and simultaneously removing some of the moisture from said ribbon, removing an additional amount of moisture from said ribbon, wrapping said ribbon around the core to form a homogeneous coating therefor, and then removing substantially all of the moisture from said coating.

14. In a machine for coating a core in strand form, a tank of liquid containing pulp, a rotatable member mounted in said tank, said member having a foraminous portion, means for straining pulp from said liquid onto said foraminous portion, means for drawing said strand around said rotatable member and into contact with the deposited material on said foraminous portion, and means for removing said pulp and core from said foraminous portion, said means comprising a moving carrier pressed against the pulp on said foraminous portion and means for forming said material to constitute a coating for the core.

15. In a machine for coating a core in strand form with pulp, a tank of liquid containing pulp, a rotatable member mounted in said tank, said member having a foraminous portion, means for straining pulp from said liquid onto said foraminous portion, means for drawing said strand around said rotatable member and into contact with the deposited material on said foraminous portion, and means for removing said pulp and core from said foraminous portion, said means comprising a moving felt pressed against the pulp on said foraminous portion and means for forming said material to constitute a coating for the core.

16. In a machine for coating a core in strand form with pulp, a tank of liquid containing pulp, a rotatable member mounted in said tank, said member having a foraminous portion, means for straining pulp from said liquid onto said foraminous portion, means for drawing said strand around said rotatable member and into contact with said foraminous portion, means for holding said strand out of contact with that section of the

foraminous portion which is near the surface of the liquid in the tank whereby pulp is strained into said section of the foraminous portion before the strand is brought into contact therewith, and means for removing said pulp from said foraminous portion, said means comprising a moving felt pressed against the pulp on said foraminous portion and means for forming said material to constitute a coating for the core. 70 75

17. In a machine for coating a core in strand form with pulp, a tank of liquid containing pulp, a rotatable member mounted in said tank, said member having a foraminous portion, means for straining pulp from said liquid onto said foraminous portion, means for drawing said strand around said rotatable member and into contact with said foraminous portion, means for holding said strand out of contact with that section of the foraminous portion which is near the surface of the liquid in the tank whereby pulp is strained onto said section of the foraminous portion before the strand is brought into contact therewith, a 80 85 90 95

rotatable felt, means for pressing said felt against the pulp on the foraminous portion whereby a continuous ribbon of pulp is transferred to the felt, means for removing the strand and said pulp ribbon from the felt, and means for forming said ribbon to constitute a coating on the core. 100 105 110 115

18. In a machine for coating a core in strand form with pulp, a tank of liquid containing pulp, a rotatable member mounted in said tank, said member having a foraminous portion, means for straining pulp from said liquid onto said foraminous portion, means for drawing said strand around said rotatable member and into contact with said foraminous portion, means for holding said strand out of contact with that section of the foraminous portion which is near the surface of the liquid in the tank whereby pulp is strained onto said section of the foraminous portion before the strand is brought into contact therewith, and means for removing said pulp and strand from said foraminous portion, said means comprising a rotatable felt pressed against the pulp on the foraminous portion, means for drawing said core around said rotatable felt and means for forming said material to constitute a coating for the core. 120 125 130

nous portion which is near the surface of the liquid in the tank whereby pulp is strained into said section of the foraminous portion before the strand is brought in said tank, said member having a foraminous portion, means for straining pulp from said liquid onto said foraminous portion, means for drawing said strand around said

5 into contact therewith, a rotatable felt, means for pressing said felt against the pulp and core on the foraminous portion, whereby a continuous ribbon of pulp is transferred to said felt, means for drawing said core around said felt and means 10 for forming said material to constitute a coating for the core.

means for drawing said strand around said rotatable member and into contact with said foraminous portion, means for holding said strand out of contact with that section of the foraminous portion which is near the surface of the liquid in the tank whereby pulp is strained onto said section of the foraminous portion, before the strand is brought into contact therewith, a rotatable felt, means 70 75

15 20 In a machine for coating a core in strand form with pulp, a tank of liquid containing pulp, a rotatable member mounted in said tank, said member having a foraminous portion, means for straining pulp from said liquid onto said foraminous portion, means for drawing said strand around said rotatable member and into contact with said foraminous portion, means for holding said strand out of contact with that section of the foraminous

20 25 30 35 40 45 50 55 60 65 70 75 80 85 90 95 100

145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000

25 portion which is near the surface of the liquid in the tank whereby pulp is strained onto said section of the foraminous portion before the strand is brought into contact therewith, a rotatable felt, means for pressing said felt against the pulp and core on the foraminous portion, whereby a continuous ribbon of pulp with the core positioned substantially at the center thereof is transferred to said felt, means for drawing said core with its attached ribbon of pulp around said felt, means for removing the core and said ribbon from said felt and means for forming said material to constitute a coating for the core.

30 90

35 95

35 100

23. In a machine for coating a core in strand form with pulp, a tank of liquid containing pulp, a rotatable member mounted in said tank, said member having a foraminous portion, means for straining pulp from said liquid onto said foraminous portion, means for drawing said strand around said rotatable member and into contact with said foraminous portion, means for holding said strand out of contact with that section of the foraminous portion which is near the surface of the liquid in the tank whereby pulp is strained onto said section of the foraminous portion, before the strand is brought into contact therewith, a rotatable

40 21. In a machine for coating a core in strand form with pulp, a tank of liquid containing pulp, a rotatable member, mounted in said tank, said member having a foraminous portion, means for straining pulp from said liquid onto said foraminous portion, means for drawing said strand around said rotatable member and into contact with said foraminous portion, means for holding said strand out of contact with that section of the foraminous portion which is near the surface of the liquid in the tank whereby pulp is strained onto said section of the foraminous portion before the strand is brought into contact therewith, a rotatable felt, means for pressing said felt against the pulp and core on the foraminous portion, whereby a continuous ribbon of pulp with the core positioned substantially at the center thereof is transferred to said felt, means for drawing said core with its attached pulp ribbon around said felt, means for squeezing moisture from said ribbon and means for wrapping said ribbon around the core to constitute a homogeneous coating therefor. 105

45 24. In a machine for coating a core in strand form with pulp, a tank of liquid containing pulp, a rotatable member mounted in said tank, said member having a foraminous portion, means for straining pulp from said liquid onto said foraminous portion, means for drawing said strand around said rotatable member and into contact with said foraminous portion, means for holding said strand out of contact with that section of the foraminous portion which is near the surface of the liquid in the tank whereby pulp is strained onto said section of the foraminous portion, before the strand is brought into contact therewith, a rotatable felt, means for pressing said felt against the pulp and core on the foraminous portion, whereby a continuous ribbon of pulp with the core positioned substantially at the center thereof is transferred to said felt, means for drawing said core with its attached pulp ribbon around said felt, means for squeezing moisture from said ribbon and means for wrapping said ribbon around the core to constitute a homogeneous coating therefor. 110

50 55 60 65 22. In a machine for coating a core in strand form with pulp, a tank of liquid containing pulp, a rotatable member mounted in said tank, said member having a foraminous portion, means for straining pulp from said liquid onto said foraminous portion, means for drawing said strand around said rotatable member and into contact with said foraminous portion, means for holding said strand out of contact with that section of the foraminous portion which is near the surface of the liquid in the tank whereby pulp is strained onto said section of the foraminous portion, before the strand is brought into contact therewith, a rotatable felt, means for pressing said felt against the pulp and core on the foraminous portion, whereby a continuous ribbon of pulp with the core positioned substantially at the center thereof is transferred to said felt, means for drawing said core with its attached pulp ribbon around said felt, means for squeezing moisture from said ribbon and means for wrapping said ribbon around the core to constitute a homogeneous coating therefor. 115 120 125 130

22. In a machine for coating a core in strand form with pulp, a tank of liquid containing pulp, a rotatable member mounted

whereby a continuous ribbon of pulp with the core positioned substantially at the center thereof is transferred to said felt, means for drawing said core and its attached pulp ribbon around said felt, means for squeezing moisture from said ribbon, means for wrapping said ribbon around the core to consti-

tute a homogeneous coating therefor, and means for removing substantially all of the moisture from said coating.

10

In witness whereof, I hereunto subscribe my name this 16th day of Feb., A. D. 1923.

HOWARD GEORGE WALKER.